

Jan. 1, 1929.

1,697,142

L. H. ROLLER

MATERIAL FOR MAGNETIC APPARATUS AND PROCESS OF MAKING SAME

Filed Nov. 21, 1925

*Fig. 1.*



*Fig. 2.*



*Fig. 3.*



*Fig. 4.*



*Fig. 6.*



*Fig. 5.*



*Fig. 7.*



INVENTOR

L. H. ROLLER

BY  
*Alfreds Bond*  
ATTORNEY

Patented Jan. 1, 1929.

## UNITED STATES PATENT OFFICE.

LOUIS H. ROLLER, OF WHITE PLAINS, NEW YORK.

## MATERIAL FOR MAGNETIC APPARATUS AND PROCESS OF MAKING SAME.

Application filed November 21, 1925. Serial No. 70,687.

My invention relates to an improved material adapted particularly for use in magnetic and electro-magnetic apparatus and to a process for making such material and it relates more particularly to a material which is mechanically strong, water proof, gas proof and in the main, a non-conductor of electricity and offering a high reluctance to the passage of magnetic lines of force, but having therein clearly defined paths of low magnetic reluctance.

It is a well known practice to pass magnetic lines of force through the walls of a sealed container to perform work within the container instead of transmitting power by means of moving mechanical elements passing through the wall with the consequent danger of leakage around such elements. However, in order to avoid serious losses due to eddy currents, such walls must be made of electrically non-conducting material. On the other hand this has heretofore limited one to the use of materials that have a high magnetic reluctance, so that the walls have had to be very thin to avoid serious losses due to leakage of magnetic flux.

It is an object of the present invention to provide a material which overcomes these objections by providing a material which is not subject to appreciable eddy current losses, in which a low magnetic reluctance is provided where desired, and which, therefore, will provide a wall of considerable thickness without entailing material losses due to magnetic leakage.

A specific use of my improved material will be found in my co-pending application, Serial No. 710,680, filed May 2, 1924, which described an electro-magnetic pump in which magnetic lines of force were passed through a sealed cylinder into an armature to reciprocate the latter and in which the cylinder was made of non-metallic material containing zones of low reluctance formed by embedding soft iron particles in the material.

It will be obvious that there would be many other uses to which the material could be applied, in certain of which it would be desirable not to form the material in cylinders but to form it in other shapes. Furthermore, if formed in cylinders certain uses would require that the regions of low reluctance be arranged transversely to the axis of the cylinder while in other cases the regions of low reluctance should be arranged parallel to the axis of the cylinder.

In producing the material I employ a woven fabric of cloth in which fine threads of soft iron or other metal of high magnetic permeability are interwoven, the wire forming stripes in the cloth. The cloth is then impregnated with certain well known phenol condensation products and built up to any desired thickness by coiling it or piling it in layers with the stripes superposed. Thereafter the coil or pile is subjected to a heat and pressure to form a bakelite or condensite mass in which the wires are embedded.

I am aware that it is not new to embed metallic wires in bakelite or condensite, a patent on such material having been granted to John M. Taylor, December 12, 1922, No. 1,438,875. However, the material described in said patent was designed with an entirely different purpose in view, viz, that of strength so that the material could be used for gears and similar mechanical elements. Such material would be entirely unsuitable for my purpose, because the metallic strands are uniformly distributed throughout the material and must necessarily be so distributed for the purpose of giving uniform strength. But it will be evident that while such material would reduce the magnetic reluctance such magnetic qualities would be uniformly distributed through the material and would defeat the purpose for which I intend to use my material. For the purpose I have in view it is essential that defined regions of low magnetic reluctance should be provided and that these regions be separated by regions of high reluctance otherwise there would be little advantage in using the material disclosed by Taylor cited, over that of using a continuous sheet or tube of iron. It is therefore, an object of my invention to provide a material in which the regions of low reluctance are separated by regions of high reluctance with no physical joint between such regions.

I also believe that I am the first to produce a fabric with separate stripes of iron wire woven therein. Heretofore, metallic wires have been interwoven with threads of textile material but the material contained wires running lengthwise as well as transversely to the material and was not confined to material in which the wires formed stripes running in one direction only.

A further object of my invention, therefore, is to provide a closely woven fabric having stripes of wire running in one direc-

tion only and to provide an efficient process for making such a fabric.

These and other objects I attain as hereinafter set forth, reference being had to the 5 accompanying drawings in which

Figure 1 is a diagrammatic perspective view of a piece of fabric provided with threads of soft metal interwoven with non-metallic threads;

10 Fig. 2 is an edge view of a sheet of my improved material showing the iron wires arranged in layers vertically alined;

Fig. 3 is a view similar to Fig. 2 representing a modified form of my material in which 15 the layers of iron wires are arranged in staggered relation to form inclined paths of low reluctance through the material;

Fig. 4 illustrates one application of my material showing in longitudinal cross section 20 a fragmentary view of a magnetically operated pump having a cylinder of my improved material, the pump being similar in form to that disclosed in the aforesaid co-pending application;

25 Fig. 5 represents another application of my material illustrating a rotary motor of induction type in which the armature of the motor is enclosed in a casing formed of my improved material, the view representing a 30 longitudinal section through a fragment of the casing with the armature of the motor indicated by broken lines;

Fig. 6 is a cross sectional view taken on the line 6—6 of Fig. 5; and

35 Fig. 7 is a diagrammatic plan view of another modification of my material illustrating how a plurality of spots of high magnetic permeability may be formed with angularly disposed layers of fabric.

40 Referring to Fig. 1, it will be observed that the fabric of which my material is composed has a warp of textile threads 10 displaced at intervals by metallic threads 11, while the weft threads 12 are all of textile material.

45 As the object of this fabric is not to attain physical strength but magnetic permeability in defined regions the wires are preferably as fine as the textile threads. In practice it has been found inadvisable to use a large number 50 of wire strands in the warp without interposing occasionally one or more textile threads between the wires. Because of the smoothness and hardness of the metallic strands the matting action which is desir-

55 able in weaving is absent, and there is a tendency for the filling threads to slide out between the warp threads while shedding. In other words, after the weft threads have been beaten into the shed by the reed, there is a 60 tendency for the filling to slide out during the shedding operation, that is, during the raising and lowering of alternate warp strands. This is prevented, however, by in-

65 troducing a thread of textile material be-

tween the wire warp threads. In practice it

is found that desirable matting can be obtained if one or more threads of textile material be introduced between every four or

five metallic threads. I therefore, form the 70 warp with stripes of metallic wires inter-

spersed with textile threads as shown at 13 in

Fig. 1. It will be understood of course, that

the stripe of iron wire need not be confined 75 to the number shown in the drawing but may

extend over any desired width of the fabric

provided warp threads of textile material are introduced at sufficiently frequent inter-

vals to produce the desired matting of the

80 fabric. Having produced the fabric shown in Fig. 1 the next step of my process is to

impregnate the fabric with a phenolic con-

densate product, after which layers of fab-

ric are arranged in a pile as shown in Fig.

2 with the stripes of metallic wire in super-

posed alined relation. The fabric may be ar-

85 ranged in a flat pile or may be wound in a

coil to form a solid rod or it may be wound

around a form, if it be desired, to produce a

cylindrical, rectangular or other form. The

pile of fabric is then subjected to pressure

90 and heat and the condensation product fills

the spaces between the textile threads and

between the wires inseparably binding all

parts together in a uniform hard substance

in which wire is thoroughly embedded. The

95 material is very strong and shows no ten-

dency to cleavage between regions of high

90 reluctance and low reluctance. The mate-

rial is also water proof and gas proof and a

good electrical insulator except where the

100 wire provides a path for electric current and,

because the wire strands are separated by the

textile threads and the impregnating con-

densate product, a high resistance to electric

current is offered, which tends in use to pre-

105 vent the formation of eddy currents. At the

same time the magnetic reluctance of the ma-

terial is markedly lowered in the zones or

regions traversed by the wires.

As explained above one of the principal

uses for which this material is adapted is to

be found in the art of refrigeration in which

it is desirable to have a closed system sealed

against gas leakage and in which mechani-

cal work may be performed by means of en-

ergy transmitted from without the system,

avoiding any moving member passing into

the system. Such an application was de-

scribed in the aforesaid co-pending applica-

110 tion and is illustrated in Fig. 4. It com-

prises a pump employing a cylinder 16

115 formed of my improved material, having

therein zones 17 of low magnetic reluctance

120 running circumferentially about the cylin-

der. The cylinder is surrounded by field coils

125 18 located in comb-shaped yokes 19, the teeth

of which engage the zones 17. Within the

cylinder 16 is a pump plunger 21 carried by a

rod 22 on which are mounted a plurality of armature sections 23 separated by collars 24, each armature section consisting of soft iron segments held in place by retaining rings 25 and tightly secured by means of wedges 26. Although condensite and bakelite are generally considered to be insoluble, I have found that they are not insoluble in anhydrous ammonia and hence, it is desirable to line the cylinder with some material, such for instance, as tin, which is not affected by ammonia when my pump is to be used for pumping ammonia gas. Such a liner is indicated at 27 and as it is not required to have any great strength, because the cylinder itself is strong enough to resist any pressures developed by the pump, it may be made merely thick enough to prevent actual contact of any liquid ammonia with the bakelite or condensite surface. The liner may be applied to the cylinder electrolytically or in any other suitable manner and as its purpose is merely to provide a coating non-soluble in the fluids handled by the pump it need not necessarily be of metal. But if a metal liner be used it should be non-magnetic so as not to divert the lines of magnetic flux passing between the yoke 19 and the armatures 23 through the zones 17. Because the material of which the cylinder is composed offers considerable reluctance to the passage of magnetic lines of force, an easier path for the flux is found through the zones 17 into and out of the armatures 23, and because of the thinness of the liner 27 there is no appreciable loss due to leakage of flux. It will be understood of course, that when the pump is to be used for pumping other gases or liquids which do not affect my improved material the liner 27 may be dispensed with.

While I have illustrated my improved material as employed with a reciprocating pump, it will be evident that it can also be used with any solenoid or any straight line motor. Fig. 5 illustrates another application in which the material is employed in connection with a rotary motor. The figure shows a cross sectional view of an induction motor with the armature removed but indicated by broken lines at 30. The field windings 31 and core 32 are separated from the armature by a casing 33 of my improved material in which bearings (one being indicated at 34) are provided for the armature shaft 35. A construction such as this can be used in refrigerating apparatus to provide rotary motion within a sealed casing transferring energy through the walls of the casing without any mechanical transmission of motion through the casing. In this application of my material, however, the regions of low magnetic reluctance must not run circumferentially about the casing but must run parallel to the axis of the armature, otherwise there would be a magnetic short circuit between the field poles and little

or no magnetic flux would reach the armature. Instead the lines of low magnetic reluctance run lengthwise of the cylindrical casing 33 as indicated at 36. In building up a casing of this sort, it will be evident that care must be exercised to arrange the layers of fabric so that the wire stripes of the outer layers will be wider than those of the inner layers, thus forming the sector shaped regions illustrated in the cross sectional view of Fig. 6. In forming the fabric it will be necessary to compute the number of wires required to effect this result. In other words, the stripes of metal must be progressively wider across the width of the fabric and must be separated by successively wider stripes of non-metallic fabric as we proceed from the inner to the outer layers. It is possible to arrange the warp of the fabric with considerable accuracy so that the successive layers will fall one above the other as the fabric is wound widthwise about a form. However, while it is desirable that the zones of low magnetic reluctance be defined transversely by radial lines, this result is not essential to the successful use of my material. For instance, there could be and in commercial practice doubtless would be, considerable irregularity along the margins of the zones, provided the principal object is maintained of producing a path of much lower reluctance through the material into the armature than exists between successive fields of poles, so that by far a greater part of the magnetic energy will pass into the armature instead of leaking across from one pole to another. It will be noted that the thickness of the casing is much greater between poles of the armature in Fig. 6 as well as between the legs of the yokes 19 of Fig. 4. My object is to provide sufficient strength by using a casing of fairly heavy thickness but this material is machined down or otherwise reduced along the zones or regions where the wire is embedded so as to reduce the thickness at these points as much as possible and thereby reduce the magnetic reluctance. At these points not only is the material reinforced by the wire therein, but it is also reinforced by the pole pieces which bear against the wire zones, so that the cylinder is not materially weakened by such reduction of thickness.

I have described the fabric of which my material is composed as having wire stripes running lengthwise or in the warp of the material. In commercial practice it is simpler to weave a fabric with wire strands in the warp rather than in the wefts, but it would be possible and in certain cases preferable to use wire in the weft rather than in the warp and hence I do not limit myself to a fabric with wire warp strands.

I have referred to the fact that it is not essential that the wire stripes of one layer be accurately superposed upon the wire stripes

of the next adjacent layer in building up my material. Indeed in some cases I find it desirable to offset the successive layers somewhat, so as to obtain the result shown in Fig. 5 3 wherein the paths of low reluctance through the material, are inclined instead of being normal to the plane of the material.

Another modification is illustrated diagrammatically in Fig. 7 which shows the 10 wire stripes of a plurality of layers of fabric, the body of the fabric being omitted. Three layers of stripes 11<sup>1</sup>, 11<sup>2</sup> and 11<sup>3</sup> are indicated, each layer forming an angle of 60 degrees with the other two. When the material is made up of layers so disposed there 15 will be intersecting spots where the magnetic reluctance is but one third of that through other parts of the material traversed by the stripes. The material may be built up of 20 any number of layers thus angularly disposed and smaller angular displacements may be used to further reduce the relative reluctance at isolated spots. In fact the layers may each be provided with a single 25 stripe or even a single wire and the successive layers be assembled with a minute angular displacement about a common intersecting point, when the transverse path of low reluctance at such point will have a relative 30 reluctance value inversely proportional to the number of the angles of displacement.

I claim:

1. A material for use in magnetic apparatus consisting of a solidified plastic substance having layers of textile fabric embedded therein, the fabric being formed with interwoven stripes of soft iron wire.
2. A material for use in magnetic apparatus consisting of a series of fabric layers bound together by a solidified phenolic condensation product, each layer including a stripe of magnetizable strands woven into the fabric.
3. A material for use in magnetic apparatus consisting of a series of fabric layers bound together by a solidified phenolic condensation product, each layer including a stripe of highly para-magnetic metal woven into the fabric.
4. A material for use in magnetic apparatus consisting of a series of fabric layers bound together by a solidified phenolic condensation product, each layer including a stripe of soft iron wire woven into the fabric.
5. A material for use in magnetic apparatus consisting of a series of fabric layers bound together by a solidified phenolic condensation product, each layer including a stripe of low reluctance wire woven into the fabric, the stripes being superposed and alined.
6. A material for use in magnetic apparatus consisting of a series of fabric layers bound together with a solidified phenolic condensation product, and each layer includ-

ing a stripe of low reluctance wire woven into the fabric, the stripe of each layer being disposed in a pre-determined geometric relation to the stripes of adjacent layers.

7. A material for use in magnetic apparatus 70 consisting of a series of fabric layers bound together by a solidified phenolic condensation product and each layer including a stripe of iron wire woven into the fabric, said stripes being disposed in superposed relation, and a 75 protective coating on the surface of the material.

8. A material for use in magnetic apparatus 80 consisting of a series of fabric layers bound together by a solidified phenolic condensation product and each layer including a stripe of iron wire woven into the fabric, said stripes being disposed in superposed relation, and a 85 non-magnetic metallic coating on the surface of the material.

9. A cylinder for use in a magnetic apparatus consisting of a length of fabric having a stripe of iron wire woven therein, the fabric being spirally wound to form a coil and the whole being bound together by a solidified 90 phenolic condensation product.

10. A cylinder for use in magnetic apparatus consisting of a hollow cylindrical coil of fabric bound by a solidified phenolic condensation product, the fabric including a circumferentially disposed stripe of iron woven into the fabric.

11. A cylinder for use in a magnetic apparatus consisting of a length of fabric having a stripe of iron wire woven therein, the fabric being spirally wound to form a hollow cylindrical coil and the whole being bound together by a solidified phenolic condensation product, and a protective coating on the inner surface of the cylinder.

12. The process of making material for magnetic apparatus which consists in weaving a fabric of textile material with stripes of metal threads interwoven therein, impregnating the fabric with a phenolic condensation 110 product, arranging the fabric in layers with the stripes in superposed and alined relation, and subjecting the whole to heat and pressure.

13. The process of making material for magnetic apparatus which consists in impregnating textile fabric with a phenolic condensation product, the fabric having stripes of metal interwoven therein, arranging the fabric in layers with the stripes of each layer disposed in a pre-determined geometric relation to the stripes of adjacent layers, and subjecting the whole to heat and pressure to solidify the phenolic condensation product.

14. The process of making material for magnetic apparatus which consists in impregnating textile fabric having stripes of metal interwoven therein, with a phenolic condensation product, arranging the fabric in layers with the stripes of the several layers disposed to superposed and alined rela- 125 130

tion, and subjecting the whole to heat and pressure.

15. The process of making material for magnetic apparatus which consists in impregnating with a phenolic condensation product a textile fabric having stripes of metal interwoven therein, winding the fabric about a form with the stripes of metal in the several coils of the winding disposed in super-

posed and aligned relation, and subjecting the whole to heat and pressure.

16. A material for use in magnetic apparatus consisting of a solidified plastic substance having layers of textile fabric embedded therein, the fabric being formed with interwoven stripes of magnetizable material.

LOUIS H. ROLLER.